

## UNITED STATES PATENT OFFICE

WALTER C. SMITH, OF MOYLAN, PENNSYLVANIA, AND PETER MACK, JR., OF LA FUNDICION, PERU, ASSIGNEES, BY DIRECT AND MESNE ASSIGNMENTS, OF ONE-HALF TO THE CERRO DE PASCO COPPER CORPORATION, OF NEW YORK, N. Y., A CORPORATION OF NEW YORK, AND ONE-HALF TO ANACONDA COPPER MINING COMPANY, OF ANACONDA, MONTANA, A CORPORATION OF MONTANA

## PROCESS FOR REFINING BISMUTH

No Drawing.

Application filed February 6, 1929. Serial No. 337,880.

Our invention pertains to the purification of bismuth metal and relates particularly to a process whereby lead and zinc may be economically removed from a bismuth alloy and 5 pure bismuth thereby obtained. Our invention relates more particularly to a process in which a molten bismuth alloy is treated with a halogen such as chlorine gas. We have discovered that, under the conditions 10 described, lead halides and zinc halides are readily formed, and are discharged from the molten metal, whereas the bismuth in the alloy is practically unaffected by the halogen until no more than a trace of lead and zinc 15 remain in the alloy.

In practise we prefer to purify bismuth alloys by passing chlorine gas through the molten mass. We have discovered that lead chloride and zinc chloride are formed and 20 eliminated before the bismuth is seriously attacked by the chlorine. The chlorides of zinc and lead are lighter than the bismuth metal and hence rise to the surface of the molten mass. If the mass is at a low temperature, these chlorides form a slag or 25 molten layer on top of the bismuth metal and very little is lost in the form of vapors. If higher temperatures are used some of the chlorides are volatilized from the bismuth 30 and slag. The fumes may be recovered in any convenient manner, for example, by water scrubbing or by the Cottrell precipitation.

In practise we prefer to conduct the chlorination at a relatively low temperature since 35 the lead chloride and zinc chloride may be recovered most easily in the form of slag. It is also advantageous to maintain a low temperature in order to avoid any volatilization of bismuth chloride such as might 40 occur during the last stages of the process. It is also frequently advantageous to commence the chlorination of the molten alloy under a slag blanket especially added, so that 45 the volatilization and loss of zinc and lead may be retarded from the start, and in order that the layer of slag may be of sufficient depth to prevent volatilization. For example we may cover over the molten alloy 50 with slag obtained from previous chlorina-

tion operations or with a mixture of molten salts such as the chlorides of sodium, potassium, lead, and/or zinc. The effect of chlorination will of course be to increase the quantity of the covering since this covering will absorb the zinc and lead chlorides formed.

The thermodynamical features of the process are indicated by the heats of formation of the chlorides as shown in the tabulation hereafter appended.

## Heats of formation

|                       | Per molecule | Per chlorine atom | 65 |
|-----------------------|--------------|-------------------|----|
| Zinc chloride.....    | 97,400       | 48,700            |    |
| Lead chloride.....    | 84,4-        | 42,220            |    |
| Bismuth chloride..... | 90,800       | 30,233            |    |

## Transition points

|                       | Melting point | Boiling point | 70 |
|-----------------------|---------------|---------------|----|
| Zinc chloride.....    | 365° C.       | 732.4° C.     |    |
| Lead chloride.....    | 498° C.       | 954.4° C.     |    |
| Bismuth chloride..... | 227° C.       | 442.2° C.     | 75 |

From the data presented it is apparent that the practicality of the process is in a large measure dependent on the relative heats of formation of the chlorides, for bismuth chloride is by far the most volatile of the three substances and, if formed, would be rapidly volatilized at a relatively low temperature.

Our experiments have indicated that an appreciable loss of bismuth does occur when the molten alloy is chlorinated at temperatures of 500-600° C.—i. e. above the boiling point of bismuth chloride. However, the process has been found to be practicable, even at these elevated temperatures, as is illustrated by the following example.

## Example I

An alloy containing 90% bismuth, 10% of lead, and 1% of zinc was melted and maintained at a temperature of 500-600° C. Chlorine gas was passed into the alloy. Fumes of metallic chlorides and excess chlorine arose from the mass and a thin layer of 100

white slag (metallic chlorides) collected on the surface of the molten metal. The chlorination was continued until the metal contained only traces of lead and zinc. In conducting the purification to this degree, 9% of the bismuth was removed, though this was found to be recoverable from the mixture of metallic chlorides.

names to this specification on the dates and at the places hereinafter indicated:—

On Mar. 9th, 1929, at New York, N. Y.  
WALTER C. SMITH.

On April 9, 1929, at La Oroya, Peru.  
PETER MACK, JR.

70

75

10 An alloy containing 75% bismuth and 25% lead was melted and maintained at a temperature of about 400° C. Chlorine was passed in, and a thick layer of lead chloride soon 15 formed on the surface of the molten mass. The chlorination was continued until only a trace of lead remained in the molten metal, the loss of bismuth (to the slag) amounting to about 3%. Subsequent to the chlorination 20 operation, the mixture was allowed to cool and the lead chloride was removed from the surface of the bismuth.

80

It may be remarked that certain metallic impurities, such as silver, antimony, and arsenic, cannot conveniently be removed by our 25 process because the chlorides of these substances have heats of formation even lower than that of bismuth chloride. These substances may be removed by other known methods. For example, the silver may be removed by the well-known "zincing process" 30 in which zinc is added to the molten alloy and the crusts of impurities formed are removed by skimming. The arsenic and antimony 35 may be removed by treating the molten metal with caustic soda, and by other known methods.

90

The presence of small quantities of impurities of the type mentioned does not interfere 40 with the operation of our process—in fact such impurities are nearly always present in the material undergoing treatment.

95

Chlorine is by far the cheapest of the halogens and for this reason we have specifically 45 described our process as it is applied with chlorine gas. It should be understood, however, that from a chemical point of view the other halogens, notably bromine, may be used to replace chlorine.

100

50 We claim:

105

1. A process for removing lead and/or zinc from a bismuth alloy which comprises heating said alloy to about 400° C. passing chlorine gas into said molten alloy, and separating 55 the resultant metallic chlorides from the purified bismuth.

110

2. A process for removing lead and/or zinc from a bismuth alloy which comprises heating said alloy to about 400° C. under slag from previous chlorinations, passing chlorine gas into said molten alloy, and separating the resultant metallic chlorides from the purified bismuth.

120

55 In testimony whereof, we have signed our

125

130